

Patented Oct. 30, 1923.

1,472,244

# UNITED STATES PATENT OFFICE.

JOHN ANDREW DALY, OF NEW ROCHELLE, NEW YORK, ASSIGNOR TO GOLD SEALED  
DENTURE PROCESS CO., INC., A CORPORATION OF NEW YORK.

## COATING.

No Drawing.

Application filed May 1, 1922, Serial No. 557,651. Renewed January 22, 1923.

To all whom it may concern:

Be it known that I, JOHN A. DALY, a citizen of the United States, residing at 5 Rochelle Park, New Rochelle, in the county of Westchester and State of New York, have invented certain new and useful Improvements in Coating, of which the following is a specification.

The invention relates to the coating of 10 vulcanite or similar plates with metals such as gold, silver, platinum, tin, etc., and has as an object the application of a metal to a plate of such material so as to be inseparable therefrom.

15 A further object of the invention is the placing of a coating of metal upon a plate of the nature mentioned in such a manner that the metal will exist not only upon the surface of the plate but to a slight extent 20 within the body thereof.

To prepare the plate for the treatment it is first thoroughly cleaned from any foreign matter, especially such as is of a 25 greasy nature, and to this end may be immersed in or scrubbed with soda or lye. The plate is then immersed in some substance which has the power of dissolving the vulcanite, as for instance chloroform, alcohol, acetic acid, or a mixture thereof, and 30 is allowed to remain therein a sufficient length of time for the material of the plate upon its surface and for a slight depth therebelow to become softened by the action of the solvent. This will 35 usually take place in about twenty minutes.

The third step in the practice of the invention is the cleansing of the plate from the solvent, for which purpose it may be merely washed with water.

40 Fourth, the plate immediately after washing is placed in an aqueous solution of gold chloride, silver nitrate, or a dissolved salt of the metal which is to be deposited thereon. In the case of silver or gold about a 45 20% solution is found to give good results. In the solution of the metallic salt about 10% of potassium sulphide ( $K_2S$ ) is dissolved and a reducing agent, such as oxalic or a tannic acid is added thereto.

50 The metallic salt in the presence of potassium sulphide and the reducing agent will cause a precipitation of the metal upon and within the plate under treatment in an exceedingly fine state of subdivision. The 55 metal seems to have an affinity for the sub-

stances supplied to the rubber for its vulcanization in such a manner as to make a close union therewith of some character, and the result as shown by the practice of the invention is a coating of metal which 60 can not be separated from the material of the plate by mechanical means.

Should the first immersion in the solution of the metallic salt with the accompanying sulphide and reducing agent give 65 an insufficient coating the plate can be a second or a third time immersed in a like solution with a resulting precipitation of fresh metal thereon at each treatment, without an additional bath in the vulcanite solvent. After sufficient metal has been deposited on the plate to make the surface thereof 70 of an electric conductor, which result may be found after the first immersion, additional metal may be deposited on the plate 75 by electroplating in the well known manner instead of by successive immersions in the solution of metallic salt.

The chemical reactions which take place in the carrying out of the invention are 80 very complex and difficult of explanation. Apparently in the presence of potassium sulphide a double sulphide of gold and potassium is formed, which sulphide is reduced by the reducing agent with the consequent precipitation of the metal upon and 85 within the body of the plate.

Minor changes may be made in the steps of the process without departing from the spirit of the invention.

I claim:

1. The process of coating a body of vulcanite with metal which comprises softening the surface of the body by chemical means and causing a precipitation of a metal upon 95 and below the softened surface of the body.

2. The process of coating a body of vulcanized rubber with a metal which comprises softening the surface of the body by treatment with a solvent, immersing the 100 body in an aqueous solution of a salt of the metal and a reducing agent, whereby the metal is precipitated upon and below the softened surface.

3. The process of coating a body of vulcanized rubber which comprises cleansing the body, treating the surface thereof with a solvent until the material of the body is 105 softened to a slight depth, removing the solvent, treating the body with an aqueous 110

solution of a metallic salt containing a reducing agent, whereby the metal in an exceedingly fine state of subdivision is deposited upon and below the surface of the body.

5. The process of coating a hard non-

metallic body with metal, which comprises exceedingly fine state of subdivision is deposited upon and below the surface of the body.

4. The process of coating a body of vulcanized rubber with metal which comprises treating the body with a solvent until the surface thereof is softened to a slight depth, removing the solvent, immersing the thus treated body in an aqueous solution of a salt of the metal, potassium sulphide, and a reducing agent whereby the metal in an

5. The process of coating a hard non-metallic body with metal, which comprises

treating the surface of the body to soften the same to a slight depth, depositing metal

in an exceedingly fine state of subdivision upon and beneath the softened surface of

the body to produce a film structurally incorporated with and overlying the surface

of the body.

JOHN ANDREW DALY.